

# UNITED STATES PATENT OFFICE.

EMIL PFIFFNER, OF FRIBOURG, SWITZERLAND.

## PROCESS OF CHEMICALLY COATING SHEETS OF CELLULOSE ESTERS WITH METAL.

No Drawing. Application filed January 11, 1923. Serial No. 612,083.

*To all whom it may concern:*

Be it known that I, EMIL PFIFFNER, citizen of Switzerland, residing at Fribourg, Switzerland, have invented certain new and useful Improvements in and Relating to a Process of Chemically Coating Sheets of Cellulose Esters with Metal, of which the following is a specification.

The application of metallic coatings to certain materials, such as for instance acetyl-cellulose, which in consequence of their great disruptive resistance and other strength are particularly suited as dielectric is meeting with all sorts of difficulties. The coating ought to adhere permanently to the material and further it has to be attached to the latter in such a manner, that the formation of any kind of air bubbles and also of a vacuum between the coating and insulating material is prevented.

The process or method according to the present invention fully satisfies these requirements. Sheets of cellulose-ester or of super-xanthogenates are chosen by way of example as the insulating material in the method hereinafter described. Even only at a thickness of  $\frac{1}{10}$  millimetre the said insulating material has given very good results.

First the cellulose-esters sheets are slightly saponified on the surface in an alkaline bath, preferably in a 2% bath of caustic potash or caustic soda.

A split-up product of the cellulose and acetic acid will be liberated by the saponification. After rinsing the sheets, preferably in running water, a metal-salt solution is applied to the saponified surfaces.

It has been discovered that the split-up product of the cellulose ester, remaining on the saponified surfaces of the sheets, acts as a reducing agent, and thus precipitates metal from the metal-salt solution.

The metal adheres to the surface prepared by the alkaline bath and forms a continuous 45 coating.

The adhesion of this metallic coating is furthered by subsequently drying the sheets at a temperature of about 100 to 150° C.

In place of the alkaline bath, for which 50 also ammonia may be employed, an acid bath may be used.

However the results obtained with the latter are not quite so good, as owing to the action of the acids the precipitated metal is 55 again dissolved in part.

Particularly silver is very good as metal deposit, but also copper and other metals may be employed.

I claim:—

1. The described process of chemically coating sheets of cellulose-esters with metal, which consists in slightly saponifying the surfaces of the sheets, rinsing them in water, and then causing a metal-salt solution to 65 act thereon, precipitating thereby reduced metal on the saponified surfaces.

2. The described process of chemically coating sheets of cellulose-esters with metal, which consists in saponifying the surfaces 70 of the sheets in an alkaline bath, and, after rinsing them in water, causing a metal-salt solution to act on the saponified surfaces, thereby precipitating reduced metal on the latter.

3. The described process of chemically coating sheets of cellulose esters with metal, which consists in superficially saponifying the sheets, rinsing them in water, causing a metal-salt solution to act on the saponified 80 surfaces and finally drying the metal-coated sheets in a temperature of about 100 to 150° C.

In testimony whereof I affix my signature.

EMIL PFIFFNER.